

## UNITED STATES PATENT OFFICE

2,186,852

PHOTOGRAPHIC SILVER HALIDE  
EMULSIONS

Gustav Wilmanns, Wolfen, Kreis Bitterfeld, and  
Wilhelm Schneider, Dessau, Germany, assign-  
ors, by mesne assignments, to Agfa Anseco Cor-  
poration, Binghamton, N. Y., a corporation of  
Delaware

No Drawing. Application November 23, 1937,  
Serial No. 176,058. In Germany December 18,  
1936

12 Claims.

(Cl. 95—6)

This invention relates to color photography and more particularly to a new and improved photographic material for color forming development.

5 In the manufacture of color transparencies and color pictures by photography and cinematography it has been proposed to use silver halide emulsions containing dyestuff components. The mode of producing the color picture differs with the nature of the dyestuff components. In 10 U. S. Patents Nos. 1,102,028 and 1,055,155 dyestuff components are used which yield dyestuff pictures with certain developers by color forming development. For producing multi-color pictures it has been proposed to cast several light-sensitive layers containing different coupling components one upon the other and in order to avoid diffusion of the coupling components the light-sensitive layers have been isolated from each other by intermediate layers. It has been shown, however, that 15 this precaution does not prevent the diffusion to the extent required by practice. The problem has been solved by using dyestuff components which are fast to diffusion and for the first time 20 a process has been attained by which a multi-layer film yields a color picture by a simple development process (see U. S. Patents 2,179,238; 2,179,244 and 2,178,612 and U. S. applications filed July 15, 1936, Ser. No. 94,340 filed August 5, 25 1936, Ser. No. 159,518 filed August 17, 1937, Ser. No. 164,499 filed September 18, 1937). Further possibilities to render dyestuff components fast to diffusion is to introduce into their molecule a sterol radical or to link up the dyestuff component molecules in a chain like manner.

This invention has for an object to provide a new range of dyestuff components with improved properties.

A further object is the provision of silver halide emulsions having incorporated the new dyestuff components fast to diffusion.

A further object is the provision of silver halide emulsions having incorporated the new dyestuff components fast to diffusion in a dis- 30 solved form.

A further object is the provision of an improved film for color photography having superposed silver halide emulsion layers, at least one of said layers containing a dyestuff component made fast to diffusion by the introduction into its molecule of a radical according to this invention.

Further objects will be seen from the detailed specification following hereafter.

The present invention is based on a process in which especially useful dyestuff formers fast to

diffusion are obtained by introducing as a substituent into a dyestuff component a compound or derivative of the cyclic menthane group. For this purpose those compounds of the said class are especially suitable which have a tendency to 5 react with the dyestuff component by means of a reactive group, for example an amino-group, an acid group, a hydroxy-group or an aldehyde group. Such compounds are, for example pinene glycol, nopolinic acid (Richter-Anschütz Chemie 10 der Kohlenstoffverbindungen II, 1935, page 263), borneol, 2-aminocamphane, camphane-2,3-diamine, 3-aminocamphor, camphor-3-carboxylic acid, camphane-3-carboxylic acid, camphyl-3-carbinol (German Patent No. 127,855), ketopinic acid (Richter-Anschütz loc. cit., page 304) or the like.

In the formulae the numbering of the positions of the camphane nucleus is as follows:



Dyestuff components into which these groups may be introduced are for example  $\alpha$ - and  $\beta$ -hydroxynaphthoic acids, 2,3-hydroxyanthracene 30 carboxylic acid, salicylic acid, hydroxy-fluorene carboxylic acid, 2,3-hydroxycarbazole carboxylic acid,  $\alpha$ -naphthol aldehyde, aminophenyl methyl pyrazolone, aromatic amines, aminonaphthols, aminonaphthol carboxylic acids, aminonaphthol sulfonic acids, aminophenols, aminobenzoyl acetic acid ester arylides, aminonaphthoyl acetic acid ester arylides, acyl acetic acid ester amino-arylides.

The dyestuff components used in the invention 40 may be added to the emulsion at any point of its production. The silver halide emulsions thus obtained are especially suitable for the purpose of color photography and may be made into layers in known manner, being applied superimposed on each other on one or both sides of a support. They may be sensitized for various regions of the spectrum. Emulsions may be applied, however, in another manner, for example the several sensitized emulsions having the different 50 dyestuff formers may be brought on to the support in the form of small particles. The emulsion layers used in the invention may be combined with other layers in which the color picture is produced by a different process, for example by 55

mordant dyeing or by toning. Furthermore, the emulsion layers of the invention may be combined with other layers which contain other dyestuff formers fast to diffusion as described in the U. S. Patent applications cited hereunder.

- The colored pictures may be produced in various manners, for example by the processes of U. S. Patents 2,179,228; 2,179,238; 2,179,244 and 2,178,612 and U. S. applications Ser. No. 94,340, filed August 5, 1936, Ser. No. 141,093 filed May 6, 1937, Ser. No. 159,518 filed August 17, 1937, Ser. No. 164,499 filed September 18, 1937 and Ser. No. 171,705 filed October 29, 1937. Thus the component located in multi-layer film may be converted into azo-dyes following development and fixing by treatment with a diazo compound such as a carbonic acid solution of tetrazotized benzidine disulfonic acid. There is thus produced in each emulsion layer together with a silver picture a dyestuff in which no structure can be perceived by magnification. The film is then treated with a silver bleaching out bath, i. e. that described in British Patent 401,340 to produce the dye image.
- The exposed emulsion layers may be developed by a simple color forming development or by a reversal development as described in U. S. Patent 2,179,234. Or the picture may be produced in multi-layer material, each layer containing one of said dyestuff components, by exposing the material, developing to black and white, in for instance Amidol, dissolving silver from the negative so produced by bleaching in for example a chromic acid bath, forming images in the remaining silver halide, developing in a developer such as is used above, forming silver halide images by treatment in a bleaching bath, i. e. again of chromic acid, forming latent images, transforming the images into silver and color images in a developer capable of forming dyestuffs with said dyestuff component, removing the developed silver and fixing in thiosulfate. In the production of color pictures the silver is generally completely removed. In the production of black-and-white pictures with the aid of the silver halide emulsion layers produced in accordance with this invention the silver may be removed or may remain in the layer.

The following examples illustrate the invention:

1. To 1 kilo of silver bromide emulsion is added a solution of 3 grams of the sodium salt of the condensation product of para-aminobenzoyl-acetyl-aniline-4-carboxylic acid with camphoric acid chloride having the following chemical formula



and the emulsion is cast to form a layer. This dyestuff former fast to diffusion may be converted into a color picture in various manners. The exposed emulsion may be developed in a solution of para-aminodimethyl-aniline, alkaline with sodium carbonate, in which case a yellow dyestuff picture is produced; or the emulsion may be exposed and the silver image developed, for example into a  $\beta$ -naphthalene-antidi-

azotate silver picture and may be subsequently immersed in a dilute acid solution, whereby a yellow picture is produced consisting of the azo-dyestuff para-camphoryl-aminobenzoyl-acetyl-aniline-4-carboxylic acid azo- $\beta$ -naphthalene.

Obviously it is also possible to produce a color picture indirectly from the silver image by, for example, tanning and hardening the gelatin under the image and then producing an azo-dyestuff picture at the non-hardened parts by introducing the layer into a diazonium solution.

2. The chloride of 2,3-hydroxynaphthoic acid is condensed with 2-aminocamphane. The condensation product has the following formula



The dyestuff former fast to diffusion thus obtained is added to a silver halide emulsion which is then converted for example with the aid of the silver antiazotate process into a picture the color of which varies with the antiazotate selected. For instance, if the antiazotate is made from dianisidine there is obtained a blue violet picture. When the anti-diazotate used is from para-nitraniline pictures of red tints are obtained.

3. 1(5'-carboxyphenyl)-3-(3'-amino-phenyl)-5-pyrazolone is condensed with the chloride of camphane-3-carboxylic acid and the compound produced is added to a silver halide emulsion. The condensation product has the following formula



When the exposed emulsion is developed by color forming development a red dyestuff image is obtained. By means of the anti-diazotate process this dyestuff former is chiefly suitable for producing yellow tints.

4. 2-hydroxyanthracene-3-carboxylic acid chloride is condensed with camphane-2,3-diamine and the product is added to a silver halide emulsion. The condensation product has the following formula



A layer of this emulsion exposed and developed is treated with a solution of tetrazotized benzidine-3,3'-disulfonic acid whereby the whole layer is uniformly dyed blue. If now the layer is further treated with the known precautions by the silver bleaching out process there is obtained on the portions free from deposited metal a blue dyestuff picture.

What we claim is:

10. 1. A silver halide emulsion for color photography containing a dyestuff component fast to diffusion, said dyestuff component being capable of forming a dye with the oxidation product of a developer and containing in its molecule a radical having substantially the chemical structure of a saturated bicyclic terpene having a dimethyl substituted carbon atom as the bridge common to the rings. 5
15. 2. A silver halide emulsion for color photography containing a dyestuff component fast to diffusion, said dyestuff component being capable of forming a dye with the oxidation product of a developer and containing in its molecule a radical having substantially the chemical structure of a saturated bicyclic terpene having a dimethyl substituted carbon atom as the bridge common to the rings. 10
20. 25. 3. A silver halide emulsion for color photography containing a dyestuff component fast to diffusion, said dyestuff component being capable of forming a dye with the oxidation product of a developer and containing in its molecule a radical having substantially the chemical structure of a saturated bicyclic terpene having a dimethyl substituted carbon atom as the bridge common to the rings, and another radical capable of preventing diffusion of said dyestuff component. 15
30. 35. 40. 4. A silver halide emulsion for color photography containing a dyestuff component fast to diffusion, said dyestuff component being capable of forming a dye with the oxidation product of a developer and containing in its molecule a radical having substantially the chemical structure of a saturated bicyclic terpene having a dimethyl substituted carbon atom as the bridge common to the rings, said dyestuff component being present in said emulsion in a dissolved form. 20
45. 50. 5. A silver halide emulsion for color photography containing a dyestuff component fast to diffusion, said dyestuff component being capable of forming a dye with the oxidation product of a developer, and capable of coupling with the formation of an azo dye, and containing in its molecule a radical having substantially the chemical structure of a saturated bicyclic terpene having a dimethyl substituted carbon atom as the bridge common to the rings. 25
55. 60. 6. A silver halide emulsion for color photography containing a dyestuff component fast to diffusion, said dyestuff component being capable of forming a dye with the oxidation product of a developer, and containing in its molecule a radical having substantially the chemical structure of a saturated bicyclic terpene having a dimethyl substituted carbon atom as the bridge common to the rings. 30
65. 7. A silver halide emulsion for color photography containing a dyestuff component fast to diffusion, said dyestuff component being capable of forming a dye with the oxidation product of a developer, and containing in its molecule an acid radical substituted by an amine of a saturated bicyclic terpene having a dimethyl substituted carbon atom as the bridge common to the rings. 35
8. A silver halide emulsion for color photography containing a dyestuff component fast to diffusion, said dyestuff component being capable of forming a dye with the oxidation product of a developer, and capable of coupling with the formation of an azo dye, and containing in its molecule a radicle selected from the class consisting of those having substantially the chemical structure of a saturated bicyclic terpene having a dimethyl substituted carbon atom as the bridge common to the rings and camphoric acid. 40
9. The emulsion as defined in claim 8, wherein the radicle is a radicle of a camphane. 45
10. The silver halide emulsion as defined in claim 8 wherein the dyestuff component is a condensation product of para-aminobenzoyl-acetyl-aniline-4-carboxylic acid with camphoric acid chloride. 50
11. The silver halide emulsion as defined in claim 8, wherein the dyestuff component is the condensation product of the chloride of 2,3-hydroxynaphthoic acid with 2-aminocamphane. 55
12. A silver halide emulsion as defined in claim 8, wherein the dyestuff component is the condensation product of a pyrazolone with the chloride of camphane-3-carboxylic acid. 60

a developer, and containing in its molecule a radical having substantially the chemical structure of a saturated bicyclic terpene having a dimethyl substituted carbon atom as the bridge common to the rings, said terpene radical being linked to the dyestuff forming radical by means of an acid amide linking. 5

6. A silver halide emulsion for color photography containing a dyestuff component fast to diffusion, said dyestuff component being capable of forming a dye with the oxidation product of a developer, and containing in its molecule an amino group substituted by a carboxylic acid of a saturated bicyclic terpene having a dimethyl substituted carbon atom as the bridge common to the rings. 10

7. A silver halide emulsion for color photography containing a dyestuff component fast to diffusion, said dyestuff component being capable of forming a dye with the oxidation product of a developer, and containing in its molecule an acid radical substituted by an amine of a saturated bicyclic terpene having a dimethyl substituted carbon atom as the bridge common to the rings. 15

8. A silver halide emulsion for color photography containing a dyestuff component fast to diffusion, said dyestuff component being capable of forming a dye with the oxidation product of a developer, and capable of coupling with the formation of an azo dye, and containing in its molecule a radicle selected from the class consisting of those having substantially the chemical structure of a saturated bicyclic terpene having a dimethyl substituted carbon atom as the bridge common to the rings and camphoric acid. 20

9. The emulsion as defined in claim 8, wherein the radicle is a radicle of a camphane. 25

10. The silver halide emulsion as defined in claim 8 wherein the dyestuff component is a condensation product of para-aminobenzoyl-acetyl-aniline-4-carboxylic acid with camphoric acid chloride. 30

11. The silver halide emulsion as defined in claim 8, wherein the dyestuff component is the condensation product of the chloride of 2,3-hydroxynaphthoic acid with 2-aminocamphane. 35

12. A silver halide emulsion as defined in claim 8, wherein the dyestuff component is the condensation product of a pyrazolone with the chloride of camphane-3-carboxylic acid. 40

GUSTAV WILMANNS.  
WILHELM SCHNEIDER.